

C. PACK.  
CASTING PROCESS.  
APPLICATION FILED MAY 14, 1919.

1,321,470.

Patented Nov. 11, 1919.



# UNITED STATES PATENT OFFICE.

CHARLES PACK, OF BROOKLYN, NEW YORK, ASSIGNOR TO DOEHLER DIE CASTING COMPANY, OF BROOKLYN, NEW YORK, A CORPORATION OF NEW YORK.

## CASTING PROCESS.

1,321,470.

Specification of Letters Patent. Patented Nov. 11, 1919.

Application filed May 14, 1919. Serial No. 296,972.

*To all whom it may concern:*

Be it known that I, CHARLES PACK, a citizen of the United States, residing at the borough of Brooklyn, in the city of New York, county of Kings, and State of New York, have invented certain new and useful Improvements in Casting Processes, of which the following is a specification.

My invention relates to processes involved in casting tubular objects which have offset or curved portions such that it would be impossible to cast the same about cores by the usual methods, and then withdraw the cores. My application, Serial No. 270,917, filed January 13, 1919, discloses and broadly claims such a process, in which the object is cast complete save for an opening, a closure then being cast in place to fill the opening. In the form of said invention specifically described and claimed in said application, a core, which by the usual practice could not be removed, is allowed to extend out through the die or mold, and thus form an opening in what should be one of the finished walls of the object, which opening is subsequently filled by casting a closure in place.

My present invention covers a modification of the specific process referred to, in which the offset portion of the tubular object is cast in place, wholly or partly, in the second operation, instead of having the offset portion cast complete at the first operation except for an opening through which a straight core extends, as in the specific process described in my said application. That is to say, in the present invention the first operation may comprise, for example, casting the main body portion and one half of the offset portion of the object, in the first operation. This may be done about a core for the main body portion of the object, which core has an offset portion at its end to form the bore of one half of the offset portion of the object. In this case the main body portion of the core need not extend through the opening which is left in the casting, but need extend only to the edge of the opening, and after the metal has been cast the core may be drawn through the opening in the axial direction of the main portion of the core. Or a core may be used for the main portion of the casting, which core may extend through the open-

ing, in order that it may be grasped to withdraw the same, and a separate core used to form the bore of one half of the offset, which core may be drawn either axially or at right angles to its axis. In either case the edge of the opening which is left may be treated, as by placing a coating of solder thereon, and the remainder of the tubular object cast in place against the treated edges, so as to make an integral structure with the original casting.

It is preferable, in this invention, that the offset portion of the object should be cast to its center line in the first operation, and the remainder in the second operation. It is only essential, however, that such arrangements be made that all cores used in both operations may be withdrawn without injuring the casting, and that the part of the casting made last may be cast against the treated edge of the part of the casting made first. In any case, a much better joint is made, when the second casting is cast against the edge of the first casting, than is possible when separately-made castings are merely soldered together at their abutting edges, in which case the joint is necessarily imperfect.

The process described herein permits interior offsets or irregular surfaces to be formed within the closed end portion and within the offset portion of the casting, which cannot be formed when a single straight core extends through an opening in an end wall, and a separate core extends into the offset, as in the specific process described in my said application, which cores must be withdrawn axially at the end of the first operation. Also when a core pin with an offset portion is used, or when the core pin for the offset portion of the casting is to be withdrawn at right angles to its own axis, a curved surface may be formed in the casting at the angle between the main portion and the offset portion of the core, by providing a suitable curved surface on the core pin or pins at this point.

In order that a clearer understanding of my invention may be had, attention is hereby directed to the accompanying drawings forming part of this application and illustrating certain ways in which my invention may be carried out. In the drawings Figure 1 is a plan view of a die show-

ing what may be termed a tone arm in process of formation therein, in cross section, with three core pins in position; Fig. 2 is a cross section taken on line 2-2 of Fig. 1; Fig. 3 is a partial plan view of the tone arm shown in Fig. 1; Figs. 4 and 5 are plan views showing further steps in the process; Fig. 6 is a front elevation partly in cross section of the completed object formed in the preceding figures; and Fig. 7 is a partial plan view similar to Fig. 1 showing a modified arrangement of core pins.

Referring to the drawings I have indicated the casting of a hollow tubular arm having a main tapering horizontal portion 1 and a pair of end portions 2 and 3 which are offset at right angles from the portion 1. Obviously, if it were attempted to cast this object as an integral construction about three cores, in one operation, it would be impossible to withdraw the core about which the portion 1 was cast. In accordance with my invention a core 4 may be used, as is shown in Fig. 1, to form the main portion 1 of the tone arm or tubular object to be cast, this core extending out of the die 5 to the left. A straight core 6 is used to form the end portion 3 of the tone arm in the usual way. A core 7 is used to form one half of the end portion 2 of the tone arm, this core pin having an operative portion 7' adapted to abut against the core pin 4 and to form what I may term the inner one half of the offset portion 2 of the tone arm.

The cores being properly positioned in the mold cavities of the die, the metal is poured, with the result that the offset portion 3 is formed, all of the main portion 1 is formed except its end closure to the left, referring to Fig. 1, and the inner or right hand one half of the offset portion 2 is formed. The metal having been poured the cores are withdrawn, the core 4 being withdrawn axially to the left and the core 7 being withdrawn either axially, or at right angles to its axis in the same direction as the core 4, which may be desirable if offsets or irregularities are to be formed within the offset portion 2 of the tone arm which would not permit the core pin 7 being drawn axially.

In the modification shown in Fig. 7 the core pin 4<sup>a</sup> is used in place of the core pin 4 just described, core pin 4<sup>a</sup> having an offset portion 7<sup>a</sup> integral therewith which takes the place of the core pin 7' shown in Fig. 1. With this construction the core 4<sup>a</sup> need not, but may, extend to the left beyond the edge 60 of the opening, and the core pin 4<sup>a</sup> with its offset portion 7<sup>a</sup> is withdrawn in the axial direction of the portion 4<sup>a</sup> thereof.

The edges of the opening 8, 8, indicated in dotted lines in Fig. 1, are now given a light coating with a molten soldering or tin-

ning mixture and the object is placed in another die 5' with another core 9 inserted in the end 2 of the object. This core 9 has its end and peripheral surfaces suitably formed to press against the portions 2 and 1 of the tone arm which have already been cast, and to form the interior surfaces of the end closure of the part 1 and the remaining portion of the offset 2. The die 5' being suitably gated as is shown at 5<sup>a</sup>, molten metal is then poured therein against the end and peripheral portions of the core pin 9 to a sufficient extent to fill the mold cavity 10 and thereby form the portions of the casting which remained to be formed. In Fig. 4 the parts are shown before the metal has been cast in the die 5', and in Fig. 5 the parts are shown after the metal has been cast, in which it will be seen that the metal 2<sup>a</sup> which has filled the mold cavity 10 completes the offset portion 2 of the casting and the end closure for the portion 1, and makes an integral construction with the portion of the casting originally made. When the metal has sufficiently solidified the core pin 9 is withdrawn axially. It is preferable to have the joint between the old and new portions of the offset 2 extend along the center line of the portion 2 as indicated, because the joint will thereby be formed in comparatively straight surfaces.

It will be obvious that a more complex structure may be formed by the application of the same principles. For example, if the offset 2 should be given an extension at an angle to the portion 2 shown in the drawings, the core pin 9 alone would not suffice in carrying out the second part of the process, an additional core pin being required to form the angularly extended part referred to, after which another core pin might have to be inserted within the bore of the extension referred to and molten metal poured about its end to fill the opening through which core pin 9 was withdrawn.

With the arrangement described a curved surface, or surface of desired configuration, may be provided in the object cast at the junction between the portion 4<sup>a</sup> and the portion 7<sup>a</sup> of the core pin. Such a curved surface is shown at 11 in Fig. 7, as cast against a suitably shaped portion of the core pin. Obviously such a surface can not be formed by the use of separate core pins such as those shown at 4 and 7 when the core pin for the offset portion of the casting must be drawn in the direction of its own axis. Such a construction is possible, however, when the core pin 7 may be withdrawn in the axial direction of core pin 4.

What I claim is:

1. A method of casting a tubular object having a straight portion closed at the end and an offset portion adjacent such end, consisting in casting such an object complete save for the end closure and part of the off-

set portion, and then casting into place the end closure and remaining part of the offset portion.

2. A method of casting a tubular object having a straight portion closed at the end and an offset portion adjacent such end, consisting in casting such an object complete save for the end closure and part of the offset portion, treating the edges of the opening thus left, and then casting into place the end closure and remaining part of the offset portion.

3. A method of casting a tubular object having a straight portion closed at the end and an offset portion adjacent such end, consisting in casting a portion of such object about a core or cores adapted to be withdrawn in straight lines, withdrawing such core or cores, and then casting into place the remainder of the object, including the end

closure and more or less of the offset portion, about a core or cores adapted to be withdrawn in straight lines.

4. A method of casting a tubular object having a straight portion closed at the end and an offset portion adjacent such end, consisting in casting the straight portion and one half the diameter of the offset portion of such object about a core or cores adapted to be withdrawn in straight lines, withdrawing such core or cores, placing molten metal on the edges of the opening thus left, and then casting into place about a core or cores adapted to be withdrawn in straight lines the remainder of the object.

This specification signed and witnessed this 12th day of May, 1919.

CHARLES PACK.

Witness:

WILLIAM R. AHRBERG.

25

30

35